

## UNITED STATES PATENT OFFICE

HERBERT L. JOHNSON, OF BROOKLYN, NEW YORK, ASSIGNOR TO STANDARD OIL  
DEVELOPMENT COMPANY, A CORPORATION OF DELAWARE

## SULFONIC LUBRICATING MATERIAL AND PROCESS OF MAKING THE SAME

No Drawing.

Application filed September 8, 1924. Serial No. 736,634.

This invention relates to improvements in lubricants of the type comprising sulfonic compounds derived from mineral oils and the like. In a preferred embodiment of the invention the lubricant contains a mineral oil sulfonic compound, an animal or vegetable oil or fat, and water. While the lubricant has many uses, it is especially advantageous in the drawing and polishing of steel, copper, brass, and nickel tubing or wire and in general to any operations in which metal is cold drawn to shape with the aid of a lubricant.

As the sulfonic compound, I may use the green sulfonic acid which is the principal organic acid occurring in the sludge formed in the treatment of petroleum lubricating oil with strong sulfuric acid. The sulfonic acid may be purified in any suitable way, if desired. Ordinarily I prefer to use sulfonic acid salts, which may be readily prepared by neutralizing the acid by a suitable base, for example sodium hydroxide. The sulfonic compound is incorporated with an oleaginous material having lubricating properties, such as animal or vegetable oils, fats, or fatty acids, especially tallow, palm oil, cocoanut oil, cottonseed oil, and oleic acid. Various other materials of this type, as well as mixtures of the same, may be used.

The following example is illustrative of the invention: For the preparation of a lubricant especially adapted for use in die-drawing metals, 15 to 30 parts of a water soluble sodium sulfonate, derived from petroleum hydrocarbons, are mixed with 1 to 15 parts of tallow and to the mixture so produced there is added sufficient water to make a total of 100 parts. For many purposes 20 parts sodium sulfonate, 5 parts tallow and 75 parts of water appear to be most satisfactory. However, I do not wish to be limited to any of the proportions stated, as these will vary with the purpose for which the lubricant is to be used. Water may be incorporated also in any desired amount. A suitable composition for die-drawing purposes is sodium sulfonate 20%, tallow 5%, water 75%.

This mixture may be prepared for use by heating, with or without agitation. The sodium sulfonate is preferably first dissolved

in water, which may be heated by steam coils or other suitable means. The tallow is then added and liquefies in the hot solution. The steam pipes may advantageously be sufficiently hot to produce some boiling in the solution. In this way proper admixture of the tallow is secured. The pipes or the like to be drawn are immersed in the hot mixture and are preferably allowed to dry after removal before being drawn. The lubricant described is an excellent drawing compound, as it gives a tough coating which is not easily displaced and has adequate lubricating properties to prevent abrasion or sticking of the rubbing surfaces.

Heating the mixture to an average temperature of 180° F. with steam coils has been found to be satisfactory, but other temperatures and means of heating may of course be employed, depending upon the particular character of the ingredients used and the results sought. Various modifications of the compositions and procedures described may also be made within the scope of the appended claims.

I claim:

1. Process of making a lubricant, comprising heating together a salt of a substantially water-soluble green sulfonic acid obtained from the sludge formed by treating petroleum lubricating oil with strong sulphuric acid, water, and a fatty oleaginous material, under conditions to effect the distribution of the latter in the water.

2. Process according to claim 1 in which the mixture is heated to about 180° F.

3. Process according to claim 1 in which the mixture is heated simultaneously producing some boiling, whereby distribution of the ingredients is effected.

4. A lubricant comprising a metallic salt of a sulfonic compound obtained from the sludge formed by treating petroleum lubricating oil with strong sulphuric acid and a non-mineral, substantially unsaponified oleaginous material.

5. A lubricant comprising a metallic salt of the green sulfonic acid obtained from the sludge formed by treating petroleum lubricating oil with strong sulphuric acid and a

normally solid, non-mineral, substantially unsaponified oleaginous material.

6. A lubricant comprising a sodium salt of the green sulfonic acid obtained from the sludge formed by treating petroleum lubricating oil with strong sulphuric acid and unsaponified tallow.

7. A lubricant comprising a sodium salt of the green sulfonic acid obtained from the sludge formed by treating petroleum lubricating oil with strong sulphuric acid 15-30 parts, and tallow 1-15 parts.

8. A lubricant comprising a sodium salt of the green sulfonic acid obtained from the sludge formed by treating petroleum lubricating oil with strong sulphuric acid 20 parts, and tallow 5 parts.

9. A lubricant comprising a salt of the green sulfonic acid obtained from the sludge formed by treating petroleum lubricating oil with strong sulphuric acid, a normally solid, substantially unsaponified lubricant material, and water.

10. A lubricant comprising a salt of the green sulfonic acid obtained from the sludge formed by treating petroleum lubricating oil with strong sulphuric acid, unsaponified tallow, and water.

11. A lubricant comprising a salt of the green sulfonic acid obtained from the sludge formed by treating petroleum lubricating oil with strong sulphuric acid 15-30%, tallow 1-15%, and water to make up to 100%.

12. A lubricant comprising a sodium salt of the green sulfonic acid obtained from the sludge formed by treating petroleum lubricating oil with strong sulphuric acid 20%, tallow 5%, and water 75%.

HERBERT L. JOHNSON.

40

45

50

55

60

65